

Aug. 8, 1961

E. R. RAMIREZ ET AL  
CONDITIONING AND ANODIZING SYSTEM

2,995,502

Filed Oct. 7, 1957

FIG. 1.



Typical Cross Sectional  
Views of Slit Aluminum  
Edges.

FIG. 2.



Original Edge  
Treated Edge (Step 1)  
Coated (Anodized) Edge (Step 2)

FIG. 3.



Cross Sectional View of  
Several Turns of Coiled  
Strip.

FIG. 4.



A - Free Access to Solution  
B - Limited Access to Solution.  
→ Electrical Current Density  
○○ GAS.

INVENTORS  
ERNEST R. RAMIREZ  
ERIK F. BARKMAN

BY Glenn & Jackson  
Their ATTORNEYS

## 1

2,995,502

**CONDITIONING AND ANODIZING SYSTEM**  
Ernest R. Ramirez, Richmond, and Erik F. Barkman,  
Henrico County, Va., assignors to Reynolds Metals  
Company, Richmond, Va., a corporation of Delaware  
Filed Oct. 7, 1957, Ser. No. 688,669  
12 Claims. (Cl. 204—15)

This invention relates to a novel method for edge conditioning and anodizing of aluminum slit sheet or strip. More particularly, the invention concerns a novel process for the manufacture of anodically coated aluminum sheet or strip possessing superior dielectric surface characteristics.

The excellent electrical properties, light weight and resistance to corrosion of aluminum have led to the widespread adoption of aluminum in sheet, strip, and foil form in the metal and electrical products industries. Properly anodized aluminum strip, for example, carries a surface layer of aluminum oxide which is capable of furnishing a dielectric coating of sufficiently high insulating power to enable the strip to be utilized as such as an electrical conductor in laminated or coil form, such as, for example, in transformers. However, anodized aluminum strip or foil has heretofore achieved only very limited application in electrical devices owing to the unependable and nonuniform character of the anodic coatings obtainable by presently known methods.

From the standpoint of the aluminum manufacturer, prior art methods for the production of oxide coated aluminum strip or sheet have been slow, cumbersome and costly. From the standpoint of the electrical products manufacturer, the available strip has been unsatisfactory and its performance uncertain, owing to poor dielectric properties both at the edges and on the main surfaces of the strip, giving rise to pinholes, rough edges, and protuberances causing short-circuiting when the material was put to use in applications such as coils, where contact was maintained directly between adjacent surfaces. Nevertheless, the dielectric advantages of an adequate and uniform coating of aluminum oxide are well known, and aluminum strip so coated would have been more extensively adopted had there been a suitable method of manufacturing sound material. Oxide insulating coatings make possible the elimination of other and separate insulation layers between adjacent aluminum surfaces when in coil form.

Aluminum sheet, strip and foil, particularly in the gages employed in electrical work, is manufactured in desired widths by conventional methods involving shearing or slitting. The nature of such operations is such as to impart to the sheared or slit edge a rough, jagged, or otherwise discontinuous aspect, such as depicted, for example, in FIG. 1 of the drawing. The overhanging, sharp edges resulting from the slitting or shearing operation, will, unless removed or modified by special treatment, adversely affect usefulness of the strip for electrical purposes. The condition of the strip edge will particularly affect the result of any anodizing operation to which the strip may be subsequently subjected in order to provide the strip with an insulating oxide coating.

In accordance with the present invention, it has been found that insulating oxide coatings of high quality, depth, and uniformity may be obtained upon the surfaces of aluminum sheet or strip by a novel process involving three treatment stages or steps. In the first step of our novel process, slit aluminum sheet or strip is subject to a treatment confined to the rough edges and contiguous portions, which has as its purpose the elimination of roughness, burrs and protuberances and the production of smooth, preferably tapered, edge portions on the strip or sheet. In the second step of the process,

## 2

the treated edges are subjected to a special edge coating operation in which the edges are anodized to build up an oxide coating thereon which serves to strengthen the edges and to protect them during the final step of the process. The third and final step of our novel process is to establish an oxide coating over the entire surface of the now preheated strip by means of an anodizing operation.

The three process steps outlined above are interrelated and cooperate to bring about a remarkably improved final anodized sheet or strip product having an oxide coating of extraordinary uniformity. The preconditioning treatment eliminates the burrs and rough edges which interfere with subsequent anodizing steps and which might otherwise cause contact and short circuiting when the finished sheet or strip is used for transformer coils or other electrical apparatus. The second or edge anodizing and precoating step serves to convert the soft and deformable edges resulting from the first or preconditioning step into difficultly bent and hard coated areas which will be protected during the final anodizing step and at the same time reduce the area over which final anodizing must be applied.

Experience has shown that when a strip is continuously anodized without any edge pretreatment, a varying rate of anodizing takes place at the slit edges as compared with the flat surface. Two factors contribute to this phenomenon. During the slitting operation, the metal on the edges is cold worked and consequently left in a high energy state and with residual stresses. As a result, the edges require a lower anodizing potential than the flat surface, causing excessive current flux or current leakage through the edges. Extremely high current densities produced at the slit edges tend to dissolve oxide formed at those edges, which are inherently more susceptible to anodizing action, almost as fast as formed, resulting in so-called burning or bare points. Another factor causing inferior formation of oxide on untreated slit edges is the fact that a metal sliver projecting at a very small angle, as shown in FIG. 1, will not anodize properly, since oxide formation takes place more or less perpendicularly to an aluminum surface, thus leaving the metal top bare. The pretreatment of step 1 of our novel process, by removing protruding metal burrs and slivers, promotes relatively uniform oxidizing of the edges in step 2. The use of step 2, in turn, enables the building up of a substantial, protective, and uniform layer of oxide on the edges, imparting good dielectric properties thereto, and preventing nonuniform oxide formation at the edges in step 3. Precoating of the edges eliminates the tendency of untreated edges to draw off anodizing current in step 3 or to concentrate it at the edges. Gradual building of an oxide coating on the metal edge prior to over-all anodizing permits increased thicknesses of oxide coatings in final anodizing, with greater uniformity and higher dielectric value.

In terms of practical plant operation, the novel process of the present invention has demonstrated that important economies in time and electrical energy are possible in the final anodizing step. Thus, a net reduction in time consumed of from 10 to 15 percent is brought about, while simultaneously, current consumption for a given area of anodized product may diminish as much as 10 percent.

For a better understanding of the invention, reference is now made to the drawing which depicts schematically the results obtainable in various stages of the process. In the drawing:

FIG. 1 depicts an untreated slit aluminum edge in cross-section;

FIG. 2 shows the effect of edge pretreatment and edge anodizing, respectively;

FIG. 3 is a cross-sectional view of adjacent turns of untreated edges in a coil of strip;

FIG. 4 depicts the action of gas formation and the distribution of current density at the coil edges.

The various steps of our novel process will now be described in detail. While the process will be described with reference to the inclusion of all three steps mentioned above, it will be understood that, where strip or sheet is available with edges in suitable condition, the first step may be omitted and that the process then comprises the novel combination of edge anodizing or pre-coating, followed by over-all anodizing.

The preconditioning or edge treatment of the first step may be performed in accordance with this invention either by electrolytic or chemical means, but preferably by electrolytic treatment. Whichever means is used, step 1 of our process involves the novel principle of limiting the electrolytic or chemical action substantially to the edges and contiguous portions and without subjecting the main flat areas of the strip or sheet to the etching, milling or polishing action. This is done preferably by subjecting the exposed rough edges to the action of the bath while the strip or sheet is in coil form. Prior to coiling, the sheet, strip or foil may be subjected to suitable alkaline or other degreasing treatments, and to water rinsing, in accordance with conventional procedures. Such degreasing and washing may, however, also be confined to the edges of previously coiled material.

In carrying out the edge treatment by electrolytic means, the principle of operation adopted is that of employing higher current densities and bath temperatures than are customary, for example, in anodizing baths. The attacking agent is preferably a mineral acid, such as, for example, sulfuric acid or fluoboric acid. Where sulfuric acid is used, the concentration may range from about 5% to 70%, but it has been found preferable to use a strength of about 30%. The temperature range may be from about 110-130° F. The current density, when using sulfuric acid, will preferably be of the order of 80 to 110 amperes per square foot of exposed edge area, while the bath temperature is maintained at a point sufficient to result in solution of any formed oxide at a rate equivalent to its rate of formation.

The rate of attack of the electrolytic solution depends upon (1) the physical condition of the metal surface, and (2) accessibility of the surface to the electrolyte.

The use, for example, of a sulfuric acid electrolyte under the conditions specified above, results in a small formation of oxide at first, but the step differs from conventional anodizing techniques, to which it may appear to bear some resemblance, in that this treatment preferentially attacks and dissolves away the sharp protruding areas, and leaves no oxide film. Burrs and rough edges which might cause metal to metal contact when the final anodized product is used for electrical coils, are eliminated, and in fact, the coiled aluminum strip or sheet is left with a unique tapered edge, as depicted in FIG. 2 of the drawing. The absence of an oxide coating at this stage leaves the metal edge with a dielectric value of substantially zero.

The use of the coiled form of aluminum strip, sheet, or foil insures limited accessibility of the attacking solution, and confines its action to the edges to be treated and the immediately contiguous areas. Electrolytic edge treatment of metals for the removal of burrs is known and is described, for example, in U.S. Patent 2,590,927. However, such treatment has heretofore been applied only to laminated products comprising layers of ferrous metal separated by intermediate layers of insulating material. Applicants were the first to discover that edge treatment for removal of burrs and rough areas could be successfully applied to aluminum in coil form with no intermediate layers of other material intervening between adjacent turns or surfaces of aluminum in the coil.

The principle of edge treatment in coil form is applica-

ble to both pretreatment of the edges, and to edge anodizing. In either case, the action of the bath is usually limited to a distance not exceeding about  $\frac{1}{8}$  of an inch from the extreme edge, with the flat portions of the coiled strip remaining dry. An example of the action resulting in a rounded or tapering edge by this method of operation is depicted in FIGS. 3 and 4. FIG. 3 illustrates the observed position and shape of the adjacent edges of several turns of coiled metal which has not been pretreated. By subjecting the edges in coil form to the action of an attacking bath, the protruding edge portions dissolve more rapidly than the other exposed areas. This is believed due to (a) higher current density at the extreme edges, and (b) entrapped liberated gas which concentrates in the crevices and tends to oppose wicking or further penetration by the bath between the metal layers. The latter effect is illustrated in FIG. 4.

The following examples serve to illustrate the step of edge pretreatment, but this phase of the invention is not to be regarded as limited thereto.

#### Example 1

A coil wound aluminum strip is immersed in the following solution and made the anode (positive), with a lead or graphite element used as the cathode; and a current is passed through the bath:

Composition----- Sulfuric acid, 30% by weight.  
Temperature----- 110-130° F.  
Current density----- 100 amps. per sq. ft.  
Time of treatment----- 5 minutes.

At the end of the time of treatment, the coil is removed from the bath, and exhibits an edge structure similar to that shown in FIG. 2.

#### Example 2

A wound aluminum coil is made the anode, with stainless steel as a cathode, in a bath having the following composition:

Composition----- Fluoboric acid, 2.5% by weight.  
Temperature----- 65-75° F.  
Tank voltage----- 12-12.5 volts.  
Time of treatment----- 5-10 minutes.

Treatment with a current under the conditions indicated results in smoothing and tapering of the edges. The coil is removed from the bath and rinsed with water to remove traces of fluoboric acid.

While the foregoing types of electrolytic pretreatments are preferred, edge polishing of wound aluminum coil may also be effected by chemical means, as illustrated by the following example:

#### Example 3

A coiled aluminum strip is immersed in a solution having the composition:

Composition----- Orthophosphoric acid (85%), 94 parts by volume. Nitric acid (60-63%), 6 parts by volume.  
Temperature----- 180-210° F.  
Time of treatment----- 3-5 minutes.

The coil is removed and washed.

The coiled strip, after receiving pretreatment of the type described in the foregoing examples, is next prepared for continuous or other types of final anodizing by means of the edge anodizing second step of our novel process.

The edge anodizing operation of step 2 of the process of this invention may be carried out either by immersing the aluminum in coil form in a suitable anodizing bath, or by unwinding the coil and passing the edge-treated strip or sheet through an edge anodizing apparatus of the type disclosed in our copending application, Serial No. 695,901, filed November 12, 1957.

The edge anodizing procedure in general comprises

immersing the material in coil form in a suitable acid anodizing electrolyte, such as sulfuric acid or oxalic acid, the coil being made the anode, with preferably a graphite cathode, and passing a current through the bath. In accordance with a preferred mode of operation of step 2, a slow build up of current density results in an oxide coating at the edges which is especially hard and abrasion resistant. When using sulfuric acid in the anodizing bath, concentration will usually be between 10 and 40% by weight, preferably about 30%, and temperature between about 30° and 80° F., depending upon desired results.

The following examples serve to illustrate edge anodizing in accordance with our invention:

*Example 4*

A wound aluminum coil, edge pretreated as described in Example 1, is immersed as anode in the following composition, using a lead cathode and a current is applied to the bath.

Composition----- Sulfuric acid, 30% by weight.  
 Temperature----- 65-75° F.  
 Current density----- 80-100 amps. per sq. ft. D.C.  
 Time of treatment----- 5 minutes.

There is obtained as a result a relatively uniform coating of oxide of about 0.003" on the exposed edges, resembling in cross-section the structure shown in FIG. 2.

*Example 5*

A preconditioned edge treated coil is immersed in a 30% sulfuric acid solution and made the anode, with a graphite cathode. Current density is slowly built up from 40 to 80 amps. per sq. ft. in the course of 1 minute. Subsequently the coil is edge anodized at 80 amps. per sq. ft. current density for 5 minutes. The dielectric value of the edge of the aluminum strip is thereby increased from about zero to about 200 volts D.C. By increasing the anodizing time from five minutes to 15 minutes, the dielectric value rises to 400-500 volts. These values are obtained in an insulation breakdown tester, using the edge of the strip (about a 2" sample) in a mercury pool, with the mercury the anode, in a D.C. arrangement.

*Example 6*

An edge-conditioned aluminum coil is made the anode in an oxalic acid electrolyte containing from 5 to 7% by weight of oxalic acid in water. Current density is gradually built up from about 10 amps. per sq. ft. to about 50 amps. per sq. ft. at a temperature of about 80° F., resulting in a dielectric value of the coil edges of about 200 volts D.C. By increasing the anodizing time, this value can be built up to any desired value below 1000 volts D.C.

*Example 7*

The edges of a wound coil are anodized in a 30% sulfuric acid bath employing a slow buildup of current density starting with about 20 amps. per sq. ft. to a figure of about 30 amps. per sq. ft. Anodization is carried on for about 5 minutes, giving a dielectric value at the edges of about 100 volts D.C. In this mode of operation the oxide coating formed is quite hard and is more resistant to abrasion than the coatings obtained in Examples 4 to 7 inclusive.

The final over-all anodizing step 3 of our novel process is applied to the material in uncoiled form in accordance with conventional methods. Thus, the coil may be unwound and passed through a regular continuous anodizing bath, employing e.g. 30% sulfuric acid at 70-80° F. In this way an oxide coating is obtained over the entire surface of the strip or sheet which is sufficiently thick and has requisite dielectric properties both at the edges and in the central portions to enable the strip to be utilized for electrical windings without the necessity of any additional insulation between adjacent turns.

While we have illustrated and described present pre-

ferred embodiments of the invention, it will be recognized that the invention may be otherwise variously embodied and practiced within the scope of the following claims.

5 We claim:

1. Process for the manufacture of anodized aluminum sheet, strip and foil, which comprises treating only the edges and contiguous portions of slit or sheared aluminum in helical coil form having rough edges in a strong acid bath to remove burrs and protuberances from said edges, then anodizing the edges and contiguous portions of said aluminum in coil form to build an oxide coating thereon, the adjacent layers of aluminum in said coil being in substantial contact with each other at said edges and contiguous portions, and thereafter anodizing said aluminum in uncoiled form to establish an oxide coating over the entire surface thereof.

2. Process for the manufacture of anodized aluminum sheet, strip and foil, which comprises electrolytically treating only the edges and contiguous portions of slit or sheared aluminum in helical coil form having rough edges in an acid bath to remove burrs and protuberances from said edges, then anodizing the edges and contiguous portions of said aluminum in coil form to build an oxide coating thereon, the adjacent layers of aluminum in said coil being in substantial contact with each other at said edges and contiguous portions, and thereafter anodizing said aluminum in uncoiled form to establish an oxide coating over the entire surface thereof.

3. Process for the manufacture of anodized aluminum sheet, strip and foil, which comprises first anodizing the edge and contiguous portions of said aluminum in helical coil form to build an oxide coating thereon, the adjacent layers of aluminum in said coil being directly in contact substantially over the interface therebetween, and then separately anodizing the central area of the aluminum to obtain a uniform oxide coating over the entire surface thereof.

4. Process for the manufacture of anodized aluminum sheet, strip and foil, which comprises treating slit or sheared aluminum in helical coil form having rough edges in a strong acid bath to remove burrs and protuberances from said edges, and then anodizing the edges and contiguous portions of said aluminum in coil form to build an oxide coating thereon, the adjacent layers of aluminum in said coil being directly in contact substantially over the interface therebetween.

5. Process for the removal of burrs and protuberances from the edges of slit or sheared aluminum sheet, strip and foil, which comprises treating the edges and contiguous portions of said aluminum in helical coil form in a strong acid bath to render said edges substantially free from burrs and protuberances, the adjacent layers of aluminum in said coil being directly in contact substantially over the interface therebetween.

6. Process for the removal of burrs and protuberances from the edges of slit or sheared aluminum sheet, strip and foil, which comprises subjecting the edges and contiguous portions of said aluminum in helical coil form to treatment in an electrolytic acid bath in which the aluminum is the anode, by passing a current through said bath to render said edges substantially free from burrs and protuberances, the adjacent layers of aluminum in said coil being directly in contact substantially over the interface therebetween.

7. Process for the removal of burrs and protuberances from the edges of slit or sheared aluminum sheet, strip and foil, which comprises subjecting the edges and contiguous portions of said aluminum in helical coil form to electrolytic treatment in a sulfuric acid bath in which the aluminum is the anode, at a temperature between about 110° and 130° F., and at a current density of about 80 to 110 amperes per sq. ft. by passing a current through said bath to render said edges substantially free from burrs and protuberances, the adjacent layers of aluminum

in said coil being in substantial contact with each other at said edges and contiguous portions.

8. Process for the edge anodizing of aluminum sheet, strip and foil, which comprises electrolytically treating only the edges and contiguous portions of slit or sheared aluminum in helical coil form having rough edges in an acid bath in which the aluminum is the anode by passing a current through said bath to render said edges substantially free from roughness, and then anodizing the edges and contiguous portions of said aluminum in coil form in a sulfuric acid bath to build an oxide coating thereon, the adjacent layers of aluminum in the said coil being in substantial contact with each other at said edges and contiguous portions.

9. Process for the edge anodizing of aluminum sheet, strip and foil, which comprises immersing said aluminum in helical coil form as the anode in a sulfuric acid bath, adjacent layers of aluminum in said coil being in substantial contact with each other at the coil edges and contiguous portions, access of said bath being limited substantially to the edges and contiguous exposed portions of the aluminum by said contact between layers, and passing a current through said bath at a temperature between about 30° and 80° F., maintaining a current density between about 80 and 100 amperes per sq. ft., to deposit an oxide coating confined to said edges and exposed portions contiguous thereto.

10. Process for the formation of a hard, abrasion-resistant oxide coating on the edges of aluminum sheet, strip and foil, which comprises immersing said aluminum in helical coil form as the anode in a sulfuric acid bath, adjacent layers of aluminum in said coil being in substantial contact with each other at the coil edges and contiguous portions, access of said bath being limited substantially to the edges and contiguous exposed portions of the aluminum by said contact between layers, and passing a current through said bath with an initial current density of about 20 amperes per sq. ft., gradually increasing the current density to about 30 amperes per sq. ft. for a period of about 5 minutes.

11. Process for the manufacture of anodized aluminum sheet, strip and foil, which comprises electrolytically treating the edges and contiguous portions of slit or sheared aluminum in helical coil form having rough edges in an acid bath to remove burrs and protuberances from said

5

10

15

20

25

25

30

35

35

40

45

edges, the aluminum being the anode in said bath, then edge anodizing said aluminum in coil form by immersing the coil as the anode in a sulfuric acid bath, adjacent layers of aluminum in said coil being in substantial contact with each other at the coil edges and contiguous portions, access of said bath being limited substantially to the edges and contiguous exposed portions of the aluminum by said contact between layers, passing a current through said bath at a temperature between about 110° and 130° F., and at a current density of about 80 to 110 amperes per sq. ft., to deposit an oxide coating confined to said edges and exposed portions contiguous thereto, and thereafter anodizing said aluminum in uncoiled form in a sulfuric acid bath at a temperature between about 70° and 80° F.

12. Process for the manufacture of anodized aluminum sheet, strip and foil, which comprises electrolytically treating the edges and contiguous portions of slit or sheared aluminum in helical coil form having rough edges in an acid bath to remove burrs and protuberances from said edges, the aluminum being the anode in said bath, then edge anodizing said aluminum in coil form by immersing the coil as the anode in a sulfuric acid bath, adjacent layers of aluminum in said coil being in substantial contact with each other at said edges and contiguous portions, access of said bath being confined substantially to the edges and contiguous exposed portions by contact of adjacent coil surfaces, passing a current through said bath with an initial current density of about 20 amperes per sq. ft., gradually increasing the current density to about 30 amperes per sq. ft. for a period of about 5 minutes to deposit a hard, abrasion resistant oxide coating on said edges, and thereafter anodizing said aluminum in uncoiled form in a sulfuric acid bath at a temperature between about 70° and 80° F.

#### References Cited in the file of this patent

#### UNITED STATES PATENTS

|           |                       |                |
|-----------|-----------------------|----------------|
| 2,057,315 | Robinson              | Oct. 13, 1936  |
| 2,094,048 | Siegel                | Sept. 28, 1937 |
| 2,374,449 | Mulcahy               | Apr. 24, 1945  |
| 2,436,227 | Phillips              | Feb. 17, 1948  |
| 2,668,936 | Robinson              | Feb. 9, 1954   |
| 2,863,796 | Theodosopoulos et al. | Dec. 9, 1958   |